

## UNITED STATES PATENT OFFICE.

GEORGE S. BROOKS, OF GARY, INDIANA.

## RETORET VOLATILIZATION OF ZINC.

No Drawing.

Application filed February 27, 1922. Serial No. 539,456.

*To all whom it may concern:*

Be it known that I, GEORGE S. Brooks, a citizen of the United States, residing at Gary, in the county of Lake and State of Indiana, have invented a new and useful Improvement in Retort Volatilization of Zinc, of which the following is a specification.

The present invention relates to methods 10 for handling zinc metal in effecting the retort volatilization thereof, such as in the process of refining zinc by distillation and in the French process of manufacturing oxide of zinc.

15 Hitherto, in handling the zinc metal for retort volatilization, it has been customary to melt and cast it into sticks or strips of a size suitable for ready introduction into the volatilizing retorts, or to melt the initially formed zinc plates and feed the zinc into the retorts in the molten condition. By introduction of the zinc metal in the methods hitherto known, a material loss of zinc is caused by oxidation and dross formation, as well as an inclusion of oxygen and oxide in the metal, which is reflected in shortened runs in the volatilizing process and in decreased life of apparatus.

20 In accordance with the present invention, the retort volatilization of zinc is carried out in the following manner:

The zinc metal to be retorted is pre-formed in sheets or plates, say, of  $\frac{1}{16}$ th to  $\frac{1}{4}$ th inch thickness, in any suitable manner, 25 for example, by electro-deposition from solutions derived from the lixiviation of suitable zinc ores. The zinc thus deposited is low in impurities, containing less than 0.07% lead.

40 The initially formed zinc plate is mechanically reduced to strips or sticks of a suitable size for introduction into the volatilizing retort, this being accomplished by means of any suitable device such as a 45 mechanical shears. The strips or sticks thus produced are preferably introduced into the furnace or retort in the manner described in my co-pending application Serial No. 539,460 $\frac{1}{2}$ , filed of even date herewith;

that is, they are retained in the heating 50 zone of the vapors issuing from the mouth of the volatilizing retort until preheated to a substantial degree before being inserted in the molten metal in the bath. They may be fed in from time to time or 55 continuously to wholly or partially replace the zinc volatilized from the retort. In carrying out the invention in connection with the French process of making zinc oxide, it is preferred that the metal or 60 spelter employed be of the character of that produced by electro-deposition from solutions derived from the ore, and containing not more than 0.07% of lead. The strips thus introduced are substantially free from 65 dross and oxide and on introduction into the retort are melted with a minimum disturbance of the working condition of the retort.

I claim:

1. A method of handling zinc in effecting the retort volatilization thereof which consists in initially forming the zinc in plates, mechanically reducing the plates into strips and feeding said mechanically formed strips of zinc into a volatilizing retort containing a molten body of zinc to replace zinc volatilized therefrom. 70

2. A method of handling zinc in effecting the retort volatilization thereof which consists in initially electro-depositing zinc in plates not over  $\frac{1}{4}$  inch thick, mechanically reducing the electro-deposited plates into strips and feeding said mechanically formed strips of zinc into a volatilizing retort containing a molten body of zinc to replace zinc volatilized therefrom. 80

3. A method of handling zinc in effecting the retort volatilization thereof which consists of initially electro-depositing zinc 90 containing less than 0.07% of lead in plates not over  $\frac{1}{4}$  inch thick, mechanically reducing the electro-deposited plates into strips and feeding said mechanically formed strips of zinc into a volatilizing retort containing a 95 molten body of zinc to replace zinc volatilized therefrom.

GEORGE S. BROOKS.